

Feb. 8, 1966

K. ZIEGLER ET AL

3,234,114

PROCESS FOR THE RECOVERY OF PURIFIED SODIUM

Filed June 27, 1962



INVENTORS

KARL ZIEGLER  
HERBERT LEHMKUHL  
WOLFRAM GRIMME

BY

*Burgess, Denklaage, Sprung*  
ATTORNEYS.

1

3,234,114

PROCESS FOR THE RECOVERY OF  
PURIFIED SODIUM

Karl Ziegler and Herbert Lehmkuhl, Mulheim (Ruhr), Germany, and Wolfram Grimme, New Haven, Conn.; said Lehmkuhl and said Grimme assignors to said Karl Ziegler

Filed June 27, 1962, Ser. No. 208,664  
Claims priority, application Germany, June 30, 1961,  
Z 8,838

12 Claims. (Cl. 204—68)

This invention relates to a process for the recovery of purified sodium.

German Patent No. 1,114,330 discloses a process in which metallic sodium is produced electrolytically with the use of electrolytes of the general formula  $MeAlR_3R'$ . In this formula,  $Me$  is sodium or a mixture of sodium and potassium,  $R$  is an alkyl radical,  $R'$  is hydrogen, an alkyl, alkoxy or aroxy radical. Readily available and particularly recommended electrolytes for this process are sodium-aluminum tetraethyl alone or in mixture with potassium-aluminum tetraethyl, preferably further modified by addition of a small amount of a sodium or potassium-alkoxy aluminum triethyl. In this process of purifying or recovering sodium, use is made of anodes which contain sodium metal and cathodes, which are inert to the sodium metal deposited at the cathode. Due to the electrolysis process, sodium metal is dissolved out of the anode material, migrates through the electrolyte and is precipitated as purified metal at the cathode and may be withdrawn at the cathode. The temperatures used in this process are preferably elevated sufficiently that the sodium metal is present in liquid form at the cathode and may be withdrawn from the cell in this form. The substantially most important application of this electrolytic recovery of sodium is the separation of sodium metal from sodium amalgam which is used as the anode material or for the electrolytic refining of raw sodium to form a particularly pure product.

The patent mentioned above gives several teachings for the practical performance of such an electrolysis. It is particularly important in practice that the sodium is precipitated in molten form and as a continuous layer at the cathode which consists of a suitable other metal, e.g. copper. A favorable course of sodium precipitation is established in most cases by electrolyzing for some time on a bright copper plate serving as the cathode. The individual droplets initially precipitated run together to form a continuous sodium film in which the sodium flows down at the cathodes which are preferably vertical or at least inclined. A special trick taught by the patent mentioned above is to provide a fabric of insulating material, e.g. a fine-meshed net of glass fibers, before the cathode plate. It has been found very surprisingly that it is possible by means of such a net of insulating material to maintain the molten sodium in suspension within the electrolyte and to prevent an undesirable sinking-down of the cathodically deposited sodium towards the anode thereby eliminating the possibility of an undesirable formation of short circuit bridges and consequently of troubles in the electrolysis.

In practical operation, electrolytic cells of this type have to meet high requirements with respect to the useful service life. The profitability of the process largely depends on how often trouble, e.g. by inner short circuits, must be expected. After troubles of this kind, the cells must be disassembled completely, the electrolyte and the cathodes must be purified, and it may even be necessary to fill in a fresh electrolyte. Only then the cell will again operate satisfactorily. When considering the fact that the electrolyte is very sensitive to air, it is obvious that

2

such restoration involves rather disagreeable and costly operations.

Continuous experiments run over a period of many months have shown that the process described has still certain deficiencies in continuous operation of an electrolytic cell. Although the process of the German patent mentioned above operates satisfactorily over relatively long periods of time, troubles must be expected in case of very long operation periods. The electrolytes described tend to precipitate traces of aluminum in addition to predominantly sodium, and then growth or clusters of spongy mixtures of aluminum and sodium occur occasionally. Moreover, metallization phenomena occur at the safety net described of insulating material when effecting the electrolysis for very extended periods of time with the use of the electrolytes mentioned so far, i.e. the net may become coated with a thin aluminum layer. However, in this case it loses the electrically insulating properties and sodium penetrates to the front side of the net so that the latter does no longer serve its purpose. Troubles of this kind may occur as early as after a few weeks of uninterrupted operation. This difficulty is of particular importance when using mixed electrolytes of potassium- and sodium-aluminum-organic complex compounds. It is known that when electrolyzing these mixtures which normally appear advantageous from general points of view, sodium is exclusively deposited at the cathode down to a minimum content of about 20% of the sodium compound. Thus, near the cathode, the electrolyte becomes poor in sodium so that troubles may occur unless constant very good intermixing of the electrolyte components is taken care of. Nevertheless, difficulties may be encountered, particularly with high current densities and, above all, when using the so-called net cathodes, because equalization of concentration within the electrolytes is aggravated within the filaments of the net itself. The individual filament of the net of a net cathode is a thread spun from many fibrillae having corresponding capillary interstices which become completely saturated or soaked with electrolyte. The portions of electrolyte which are bound in these interstices and subjected to the direct electrolytic decomposition mix only difficultly with further portions of the electrolyte bath. Thus, it appears that this may involve a serious cause of undesirable troubles.

It is urgently desirable for all of these reasons to develop an electrolyte which, while having a correspondingly high conductivity in the prior art process mentioned above, contains only sodium as cations and which does not give rise to the troubles described above.

The invention consists in the finding that cells for the electrolytic recovery of sodium from an anode material which contains sodium metal, e.g. from sodium amalgam or raw sodium, can be operated for many months without any trouble when using a mixture of sodium-aluminum tetraethyl and sodium-aluminum tetramethyl as the electrolyte. The mole ratio of the components of this mixture is preferably about 1:1 but may deviate to both sides by a certain amount. The limits are at 30 to 75 mole percent  $NaAl(CH_3)_4$  and 70 to 25 mole percent of  $NaAl(C_2H_5)_4$ .

The conductivity of an exactly equimolar mixture of the two complex compounds at  $130^\circ C$ . is  $10 \times 10^{-2}$  ohms $^{-1}$  cm. $^{-1}$ , i.e. the conductivity is very good. Moreover, the mixture of sodium-aluminum tetramethyl and sodium-aluminum tetraethyl melts at very low temperatures with the unusually low eutectic of  $83^\circ C$ . leading to completely liquid electrolyte mixtures already at temperatures in the neighborhood of  $100^\circ C$ .

The accompanying drawing indicates these relationships. In the drawing:

The figure is a plot of melting points for mixtures of  $\text{NaAlEt}_4$  and  $\text{NaAl}(\text{CH}_3)_4$ .

In practical operation, the electrolytes are preferably mixed with a small amount of the corresponding sodium-alkoxy aluminum trialkyl compound. A few percent are sufficient so that the conductivity is reduced to an unimportant extent only. This measure reliably protects the cathodically deposited sodium from co-deposition of aluminum. The alkoxy triethyl or trimethyl compound may be added most conveniently by adding a corresponding amount of any alcohol to the mixture of the two tetraalkyl complexes. The temperatures to be maintained during electrolysis must range above the melting point of sodium. Most preferred are temperatures between about 100° and 120° C., but temperatures up to about 160° C. may be used.

The preparation of sodium-aluminum tetraethyl which is one component of the process of the invention is sufficiently described in literature. The other component, i.e. sodium-aluminum tetramethyl, may, for example, be prepared by one of the processes described below.

#### EXAMPLE 1

50 grams (=2.18 gram atoms) of sodium are heated to 180° C. in a dry 1 liter three-necked flask filled with inert gas and equipped with a stirrer, a reflux condenser and a dropping funnel. While stirring, 100 mls. (=96 gms. =1.04 moles) of  $\text{Al}(\text{CH}_3)_2\text{Cl}$  are dropped onto the molten sodium. When all of the aluminum dimethyl chloride has been added, the pulverulent reaction mixture is allowed to cool while stirring. Then 300 ml. of dry diethyl ether are added and the mixture is stirred for about 20 minutes. After having stopped the stirrer, the solid products ( $\text{NaCl}$  and aluminum) are allowed to settle, the clear ether solution of  $\text{NaAl}(\text{CH}_3)_4$  is withdrawn by siphoning, and the residue is extracted three times with 200 ml. of ether. After removal of the ether by distillation and drying under a vacuum of  $10^{-3}$  mm. Hg the combined solutions give 55 gms. (=0.5 moles) of  $\text{NaAl}(\text{CH}_3)_4$ . Analysis of the substance gives the following values:

Found: Na, 20.95; Al, 24.6;  $\text{CH}_3$ , 54.2. Calculated: Na, 20.9; Al, 24.6;  $\text{CH}_3$ , 54.6. The yield is 96.5%.

#### EXAMPLE 2

$\text{NaAl}(\text{CH}_3)_4$  can be prepared in the same manner as described in Example 1 by allowing 48.3 gms. (=0.67 mole) of  $\text{Al}(\text{CH}_3)_3$  to drop into 11.5 gms. (=0.5 gram atoms) of molten sodium at 180–200° C. The yield and purity of the product are similarly good as those in Example 1.

#### EXAMPLE 3

9.7 gms. (=58.4 millimoles)  $\text{NaAlEt}_4$  are dissolved in 50 ml. benzene at 70° C. while stirring. A solution of 5.6 gms. (=78 millimoles)  $\text{Al}(\text{CH}_3)_3$  in 20 ml. benzene is dropped into the solution. A white insoluble precipitate is formed immediately. The reaction mixture is stirred for another hour and then the precipitate is filtered off while taking the precautionary measures usual for handling air- and moisture-sensitive organometallic compounds. The precipitate is dried at  $10^{-3}$  mm. Hg and 150° C. The resultant 6.2 gms. (=56.3 millimoles)  $\text{NaAl}(\text{CH}_3)_4$  are analytically pure. The yield is 96.5% of the theoretical.  $\text{NaAl}(\text{CH}_3)_4$  melts at 238° C. without decomposition.

Other very simple methods of preparing the mixtures of sodium-aluminum tetramethyl and ethyl of the invention are to add the necessary amount of sodium-aluminum tetramethyl to molten sodium-aluminum tetraethyl with exclusion of air or to dissolve both substances in air-free and dry diethyl ether or tetrahydrofuran and to evaporate these solutions to dryness. It is also possible to combine the production of the mixtures directly with the preparation of the alkali-aluminum tetraalkyl compounds. This is described in the following examples.

#### EXAMPLE 4

The procedure is initially the same as that described in Example 3. However, the precipitate of sodium-aluminum tetramethyl is not filtered off but 1.9 gms. of sodium hydride which is preferably in the form of a 20% suspension in a mineral oil is added to the reaction mixture which still contains free aluminum triethyl. After stirring for about 1 hour at 100° C., the mixture is filled into an autoclave of 200 ml. capacity while excluding the air; ethylene is introduced until a pressure of 20 kgs./cm.<sup>2</sup> is reached and the mixture is heated to 160° C. while shaking. The ethylene is taken up rapidly. As soon as the pressure remains constant, the temperature is allowed to drop to 100° C., the excess ethylene is released, and the liquid contents are withdrawn from the autoclave with exclusion of air. The liquid forms two layers, the upper one being practically only the mineral oil introduced by the sodium hydride, the lower layer being a mixture according to the invention comprising sodium-aluminum tetraethyl and sodium-aluminum tetramethyl in a mole ratio of 4:3.

#### EXAMPLE 5

In the manner described in Example 1, a mixture of 48 gms. (=0.5 mole)  $\text{Al}(\text{CH}_3)_2\text{Cl}$  and 60 gms. (0.5 mole)  $\text{Al}(\text{C}_2\text{H}_5)_2\text{Cl}$  is allowed to drop at about 150° C. onto 50 gms. (=2.18 gram atoms) of molten sodium while stirring. After cooling, 300 ml. of dry diethyl ether are added to the reaction mixture which is then stirred about 20 minutes. After having stopped the stirrer, the solid products, i.e.,  $\text{NaCl}$  and aluminum, are allowed to settle. The clear ether solution is siphoned off and the residue is again extracted with about 200 ml. of ether. The combined ether solutions give 69 gms. of a mixture of  $\text{NaAl}(\text{CH}_3)_4$  and  $\text{NaAl}(\text{C}_2\text{H}_5)_4$  in a mole ratio of 1:1 after having distilled off the ether and dried the residue under a vacuum of  $10^{-3}$  mm. Hg. This reaction product melts at 83° C. The yield is substantially quantitative.

#### EXAMPLE 6

The equimolar mixture of  $\text{NaAl}(\text{CH}_3)_4$  and  $\text{NaAl}(\text{C}_2\text{H}_5)_4$  can be prepared in a manner similar to that described in Example 5 by allowing an equimolar mixture of  $\text{Al}(\text{CH}_3)_3$  and  $\text{Al}(\text{C}_2\text{H}_5)_3$  (0.67 mole each) to drop onto 23 gms. (=1 gram atom) of molten sodium. The reaction mixture is processed in a manner analogous to that described in Example 5.

#### EXAMPLE 7

457 gms. (=5 miles)  $\text{Al}(\text{CH}_3)_2\text{Cl}$  are heated to about 80 to 90° C. in a dry 1000 ml. flask provided with a stirrer and reflux condenser and filled with inert gas. Then 600 gms. of a 20%  $\text{NaH}$  suspension in paraffin oil (containing 120 gms.  $\text{NaH}$  (=5 moles)) are carefully added by siphoning, following which the reaction mixture is stirred for about 1 hour until halogen is no longer contained in the solution. After cooling, the reaction mixture is separated from precipitated  $\text{NaCl}$  by centrifuging and filled into a 2 liter autoclave while taking the known precautionary measures usual for handling air- and water-sensitive organometallic compounds. The contents of the autoclave are heated to about 60–70° C. while shaking or rotating the reaction vessel following which 10 to 20 atmospheres of ethylene are introduced under pressure. The initially rapid pressure drop necessitates frequent supply of additional ethylene until the pressure remains constant after about 45 minutes. After having vented the excess ethylene, 600 gms. of the 20%  $\text{NaH}$  suspension (containing 120 gms.  $\text{NaH}$  = 0.5 mole) are introduced into the autoclave and the autoclave is shaken or tumbled for about 15 to 30 minutes at 80 to 100° C. until all of the  $\text{NaH}$  has dissolved, which is verified by sampling after 30 minutes. Then 20 atmospheres of ethylene are introduced under pressure and the contents of the autoclave are heated to 160° C. The ethylene con-

sumed by the reaction is made up by repeatedly introducing ethylene under pressure. The pressure drop ceases after 2 to 3 hours and the reaction is completed.

After having vented excess ethylene, the contents of the autoclave, while still liquid, i.e. at a temperature above 90° C., are siphoned into a dry 2 liter flask filled with an inert gas. At 90° C., the reaction product is a liquid system comprising two phases. The upper layer is paraffin oil which is substantially free from organometallic compounds and siphoned off from the lower phase. The lower layer is a mixture of  $\text{NaAl}(\text{CH}_3)_4$  and  $\text{NaAl}(\text{C}_2\text{H}_5)_4$  in a mole ratio of 1:1 which solidifies at 80° C. with formation of crystals. The yield of this mixture is 650 gms. (95% of the theoretical).

#### EXAMPLE 8

Into a 10 liter vessel with stirrer, there are placed a suspension of 1 kg. aluminum grit and a mixture of  $\text{AlEt}_2\text{Cl}$  and  $\text{AlMe}_2\text{Cl}$  in a molar ratio of 1:1 in amount sufficient that the mixture is still well stirrable. The reaction vessel is heated to 105–115° C. and an equimolar mixture of ethyl chloride and methyl chloride in liquid form (from an inverted stock bottle) is introduced through a capillary extending down to the bottom of the vessel. It is also possible to introduce ethyl chloride and methyl chloride in equal amounts separately through two capillaries. The addition of the alkyl halides is effected at a rate sufficient that the temperature is maintained between 105° C. and 115° C.

Alkyl chloride in amount of between 350 and 700 grams is taken up within one hour. 3 kgs. of the mixture of alkyl halides and all of the aluminum charged are reacted within about 6 hours. The conversion of the resultant mixture of methyl and ethyl aluminum sesquichlorides into  $\text{Al}(\text{CH}_3)_2\text{Cl}$  and  $\text{Al}(\text{C}_2\text{H}_5)_2\text{Cl}$  or  $\text{Al}(\text{CH}_3)(\text{C}_2\text{H}_5)\text{Cl}$  is effected as follows: 425 gms. of sodium are molten in a second 10 liter reaction vessel. The reaction mixture of the alkyl aluminum sesquichlorides is allowed to drop onto the sodium at about 110° C. while stirring. After all of the mixture has been added, stirring is continued for about 30 minutes. Following this, the resultant



is distilled off from the sodium chloride and aluminum at a bath temperature which must be increased to 200° C. towards the end of the distillation.

There are obtained 2.5 kgs.  $\text{Al}(\text{CH}_3)(\text{C}_2\text{H}_5)\text{Cl}$ , i.e. 83% of the theoretical yield.

The complex mixture  $\text{NaAl}(\text{CH}_3)_4$ – $\text{NaAl}(\text{C}_2\text{H}_5)_4$  is prepared in a manner analogous to that of Example 1 by allowing the reaction mixture having the composition  $\text{Al}(\text{CH}_3)(\text{C}_2\text{H}_5)\text{Cl}$  and obtained in Example 8 to drop onto the corresponding amount of molten sodium. There is obtained the 1:1 molar mixture  $\text{NaAl}(\text{CH}_3)_4$ – $\text{NaAl}(\text{C}_2\text{H}_5)_4$  in a good yield.

#### EXAMPLE 9

The electrolytic cell used consists of a cylindrical and internally enamelled steel kettle which contains at the bottom raw sodium to be refined as a melt. Suspended in the kettle is a cylinder of enamelled sheet steel of somewhat smaller diameter, which is open at both ends and has horizontally tightened across the lower opening a wide-meshed glass fiber fabric having a mesh size of 1 to 3 mm. The net is arranged at a distance of 3 to 5 mm. above the surface of the liquid sodium. Arranged closely above the net is a net of copper or iron wire as the cathode.

The electrolysis temperature is 150° C. A mixture of sodium-aluminum tetraethyl and tetramethyl in a 1:2 molar ratio is used as the electrolyte. The level of the molten electrolyte must be above the upper edge of the suspended cylinder, so that the sodium deposited at the cathode is surrounded by the electrolyte from above and below. An electrode current density of 20 a./dm.<sup>2</sup> can be

maintained at a terminal voltage of 1.1 v. The cathodically formed sodium collects above the glass fiber net and may be drained from this space from time to time. Care is taken by the addition of raw sodium during the electrolysis that the distance between the anode and cathode is kept constant.

Under the conditions described above, the electrolytic refining of raw sodium can be carried out continuously for months without any trouble. Test runs were operated for more than six months. In contrast, test runs effected with electrolytes containing only ethyl groups had to be discontinued after 3 to 4 weeks due to troubles in the sodium deposition. The same difference is suitability of the electrolyte systems was also found in test runs which were effected for an extended period of time with the use of sodium amalgam as the anode (see Example 10 below).

The yield of sodium is 23 grams per 26.8 amperes-hours, and 23 grams of Na were dissolved anodically by the same amount of current. The yield is 100%.

20

#### EXAMPLE 10

The procedure is the same as that described in Example 9, except that the same volume of 1% sodium is substituted for the molten raw sodium. Electrolysis is effected at 150° C. with a current density of 30 a./dm.<sup>2</sup> at a terminal voltage of 1.7 v. The sodium deposited at the cathode collects as a continuous liquid layer above the net of glass fiber fabric. To remove the joulean heat and for mixing the electrolyte, a greater electrolyte stock is recirculated through the electrolytic cell while maintaining the liquid in the electrolytic cell at a constant level. This is easily accomplished by allowing an equal volume of electrolyte per unit time to flow from a stock vessel into the space between the anode and cathode as that pumped back into the stock vessel from a point opposite of the inlet opening. The amount of sodium deposited cathodically after 185 amperes-hours is 160 grams. The Na content of the initial Na amalgam which was 1% has been reduced to about 0.2%. The amalgam is preferably removed from the cell and may be used for another electrolysis after having been concentrated to 1% Na.

In this experiment, the same current density (30 a./dm.<sup>2</sup>) with about the same voltage (1.5–1.7 v.) is achieved as it would be obtained with an electrolyte mixture of 80%  $\text{KAlEt}_4$  and 20%  $\text{NaAlEt}_4$  under otherwise identical conditions.

#### EXAMPLE 11

The procedure is the same as that described in Example 10 except that an electrolyte mixture of  $\text{NaAl}(\text{C}_2\text{H}_5)_4$  and  $\text{NaAl}(\text{CH}_3)_4$  in a 1:1 molar ratio is used. A terminal voltage of about 1.5 to 1.7 v. is required at a current density of 20 a./dm.<sup>2</sup>

What is claimed is:

55 1. A process for the recovery of purified sodium which comprises passing an electrolysis current between a cathode and an anode through an electrolyte containing a mixture of sodium aluminum tetramethyl and sodium aluminum tetraethyl, said anode being a sodium metal containing electrode and said cathode being inert to the cathodically deposited sodium, to electrolyze sodium from the anode and deposit sodium at the cathode, the sodium electrolyzed at the anode replacing in the electrolyte sodium deposited at the cathode, and recovering the purified sodium so formed.

60 2. The process of claim 1 wherein said electrolyte comprises from 30 to 75 mole percent of  $\text{NaAl}(\text{CH}_3)_4$  and from 70 to 25 mole percent of  $\text{NaAl}(\text{C}_2\text{H}_5)_4$ .

65 3. The process of claim 1 wherein said electrolyte comprises about equivalent amount of  $\text{NaAl}(\text{CH}_3)_4$  and  $\text{NaAl}(\text{C}_2\text{H}_5)_4$ .

70 4. The process of claim 1 wherein said electrolyte additionally contains small amounts of a corresponding alkoxy complex compound.

75 5. The process of claim 1 which includes effecting said

electrolysis with said cathode in a cathode space and said anode in an anode space while maintaining said cathode space and said anode space separated by a diaphragm formed of an insulating material.

6. The process of claim 1 wherein the sodium aluminum tetramethyl component of said electrolyte is prepared by reacting aluminum trimethyl with sodium metal. 5

7. The process of claim 1 wherein the sodium aluminum tetramethyl component of said electrolyte is prepared by reacting a member selected from the group 10 consisting of  $Al(CH_3)_2X$ ,  $Al(CH_3)X_2$ , wherein X is halogen, and mixtures thereof with sodium metal.

8. The process of claim 1 wherein the sodium aluminum tetramethyl component of said electrolyte is prepared by reacting aluminum trimethyl with a sodium 15 aluminum tetraalkyl compound wherein alkyl contains at least two carbon atoms.

9. The process of claim 1 wherein the electrolyte is maintained at a temperature of between about 100 and 160° C. 20

10. The process of claim 1 wherein one of the components of said electrolyte mixture is prepared in the presence of said other component.

11. The process according to claim 1, wherein the electrolysis is effected with said anode as a lowermost layer, the electrolyte as the middle layer and the cathodically deposited sodium kept in suspension by a wide mesh net of insulating material as the uppermost layer.

12. Process according to claim 11, wherein the net comprises threads formed of filaments.

#### References Cited by the Examiner

##### UNITED STATES PATENTS

|           |        |                |        |
|-----------|--------|----------------|--------|
| 2,849,349 | 8/1958 | Zeigler et al. | 204-59 |
| 2,952,589 | 9/1960 | Zeigler et al. | 204-59 |
| 2,985,568 | 5/1961 | Zeigler et al. | 204-59 |
| 3,028,323 | 4/1962 | Kobetz         | 204-68 |

##### FOREIGN PATENTS

864,393 4/1961 Great Britain.

JOHN H. MACK, Primary Examiner.

JOHN R. SPECK, Examiner.